

## UNITED STATES PATENT OFFICE

2,191,977

## TREATMENT OF STAPLE FIBER

Fritz Schneider, Hans Altgelt, and Wilhelm Neugebauer, Wiesbaden-Biebrich, Germany, assignors to Kalle & Co. Aktiengesellschaft, Wiesbaden-Biebrich, Germany

No Drawing. Application December 17, 1937, Serial No. 180,328. In Germany December 23, 1936

5 Claims. (Cl. 28—1)

This invention relates to staple fiber (cellulose wool, in German=Zellwolle) which consists of regenerated cellulose, or materials consisting of or containing such staple fiber for example yarns or fabrics. Primarily it relates to viscose staple fiber.

An object of the present invention is a new process for treating staple fiber which process improves the staple fiber. The new process is applicable not only to the treatment of materials made of staple fiber alone, but also to any spun or woven goods containing staple fiber, particularly to mixed fabrics which contain wool or cotton in addition to staple fiber. Another object of the invention are staple fiber materials improved by the new process.

The new process consists in causing to act on the staple fiber material a solution of an enzyme preparation such as is obtained with the aid of a bacterium selected from the group consisting of *Bacillus subtilis* and *Bacillus mesentericus*, the solution being substantially free from the said bacteria. The production of such products is described, for example in German specification 320,571. The preferable procedure is to treat the fabric with an enzyme solution as hot as possible, for example at 70—80° C. The solution may contain suitable additions, for instance activators, buffer substances or the like.

The improvement produced by the process shows itself in the first place in an improvement in the capacity of the staple fiber or the material containing it for being dyed. Without the pre-treatment afforded by this invention it is generally difficult to dye staple fiber throughout in a manner free from objection and uniform with, for example, substantive dyestuffs, indanthrene dyestuffs and other vat dyestuffs. When the process of the invention is applied, there are obtained uniform pure tints. In addition, the new process in general brightens the goods and improves greatly the feel of the staple fiber so that the goods acquire a full soft feel.

The staple fiber may be treated with the enzymes at any stage of its working up, for example in the form of hanks or in the form of finished fabric. At the same time, the material may be treated with wetting agents, emulsifying agents, cleansing agents or the like, for example with condensation products of fatty acid chlorides of high molecular weight with aminocarboxylic acids, aminosulphonic acids or oxysulphonic acids. Such products are, for instance N-oleyltaurine and N-stearyl-sarcosine. There also come into question, for example, polyglycol ethers of alcohols of high molecular weight or phenols, for instance iso-octylphenol.

The following example illustrates the invention:

A fabric consisting solely of staple fiber is treated at 75° C. with a neutral liquor containing per litre 5—10 grammes of a commercial bacterial enzyme preparation obtained with the aid of *Bacillus mesentericus*, for instance, the so-called "Biolase". The treatment may advantageously be on the Foulard apparatus. After some minutes the impregnated goods are rolled up and laid aside. In this condition they remain for some hours, preferably over night, and are finally rinsed hot (about 80° C.). The goods thus treated have a full soft feel and can be dyed especially well with dyestuffs coming into question for such material, for example substantive dyestuffs. When a material which has been sized with starch is treated in the manner described, the size is simultaneously removed.

We claim:

1. The process which consists in treating staple fiber material made of regenerated cellulose with a solution of an enzyme preparation obtained with the aid of a bacterium selected from the group consisting of *Bacillus subtilis* and *Bacillus mesentericus*, the solution being substantially free from the said bacteria.

2. The process which consists in treating staple fiber material made of regenerated cellulose with a solution of an enzyme preparation obtained with the aid of a bacterium selected from the group consisting of *Bacillus subtilis* and *Bacillus mesentericus* at a temperature of at least 70° C., the solution being substantially free from the said bacteria.

3. The process which consists in treating staple fiber material made of regenerated cellulose with a solution of an enzyme preparation obtained with the aid of a bacterium selected from the group consisting of *Bacillus subtilis* and *Bacillus mesentericus* at 70 to 80° C., the solution being substantially free from the said bacteria.

4. The process according to claim 1 wherein the said staple fiber material is a fabric containing staple fiber.

5. An improved staple fiber material made from regenerated cellulose which has been treated with the solution of an enzyme preparation obtained with the aid of a bacterium selected from the group consisting of *Bacillus subtilis* and *Bacillus mesentericus*, the solution being substantially free from the said bacteria and which has an improved affinity to dyestuffs and a full and soft feel.

FRITZ SCHNEIDER.  
HANS ALTGELT.  
WILHELM NEUGEBAUER.